



US009720356B2

(12) **United States Patent**  
**Ota et al.**

(10) **Patent No.:** **US 9,720,356 B2**  
(45) **Date of Patent:** **\*Aug. 1, 2017**

(54) **IMAGE FORMING APPARATUS AND IMAGE FORMING METHOD**

(71) Applicant: **FUJI XEROX CO., LTD.**, Tokyo (JP)

(72) Inventors: **Naoki Ota**, Kanagawa (JP); **Katsuyuki Kitajima**, Kanagawa (JP); **Nagahito Ichijo**, Kanagawa (JP)

(73) Assignee: **FUJI XEROX CO., LTD.**, Minato-ku, Tokyo (JP)

(\*) Notice: Subject to any disclaimer, the term of this patent is extended or adjusted under 35 U.S.C. 154(b) by 0 days.

This patent is subject to a terminal disclaimer.

(21) Appl. No.: **14/941,019**

(22) Filed: **Nov. 13, 2015**

(65) **Prior Publication Data**

US 2016/0349674 A1 Dec. 1, 2016

(30) **Foreign Application Priority Data**

May 29, 2015 (JP) ..... 2015-110342

(51) **Int. Cl.** **G03G 15/20** (2006.01)

(52) **U.S. Cl.** CPC ..... **G03G 15/20** (2013.01)

(58) **Field of Classification Search**

None

See application file for complete search history.

(56) **References Cited**

U.S. PATENT DOCUMENTS

7,056,638 B1 6/2006 Tomita et al.  
9,354,558 B1 \* 5/2016 Ota ..... G03G 15/1605

|                   |         |                |                          |
|-------------------|---------|----------------|--------------------------|
| 9,367,001 B1 *    | 6/2016  | Kitajima ..... | G03G 15/2017             |
| 9,529,291 B2 *    | 12/2016 | Ota .....      | G03G 9/0819              |
| 9,547,256 B2 *    | 1/2017  | Ota .....      | G03G 15/0865             |
| 2005/0220506 A1 * | 10/2005 | Nakayama ..... | G03G 15/2025<br>399/323  |
| 2007/0166635 A1 * | 7/2007  | Yamamoto ..... | G03G 9/0819<br>430/108.8 |
| 2009/0148785 A1   | 6/2009  | Yogome         |                          |

FOREIGN PATENT DOCUMENTS

|                  |        |
|------------------|--------|
| JP 2004-145243 A | 5/2004 |
| JP 2011-158758 A | 8/2011 |
| JP 5125959 B2    | 1/2013 |

\* cited by examiner

*Primary Examiner* — David M Gray

*Assistant Examiner* — Thomas Giampaolo, II

(74) *Attorney, Agent, or Firm* — Sughrue Mion, PLLC

(57) **ABSTRACT**

An image forming apparatus includes a developing unit that stores a developer containing a toner and develops an electrostatic charge image on a image holding member by the developer to form a toner image, a transfer unit that transfers the toner image on the image holding member onto a recording medium, and a fixing unit that performs an operation of heating and pressing twice or more to the toner image on the recording medium by at least one heating and pressing member which contacts with the toner image, wherein the toner has a sea and island structure of a sea portion containing a binder resin and an island portion containing a release agent, a maximum frequent value and a skewness in distribution of eccentricity B of the island portion is 0.75 to 0.95 and -1.10 to -0.50, respectively, and eccentricity B is defined in the specification.

**11 Claims, 3 Drawing Sheets**



FIG. 1



FIG. 2



FIG. 3



FIG. 4



## IMAGE FORMING APPARATUS AND IMAGE FORMING METHOD

### CROSS-REFERENCE TO RELATED APPLICATIONS

This application is based on and claims priority under 35 USC 119 from Japanese Patent Application No. 2015-110342 filed May 29, 2015.

### BACKGROUND

#### 1. Technical Field

The present invention relates to an image forming apparatus and an image forming method.

#### 2. Related Art

A method of visualizing image information, such as an electrophotographic method has been used in various fields. In the electrophotographic method, an electrostatic charge image is formed as image information on a surface of an image holding member by performing charging and forming the electrostatic charge image. Developing is performed by using a developer containing a toner so as to form a toner image on the surface of the image holding member. The toner image is transferred to a recording medium, and then the toner image is fixed on the recording medium. Thus, the image information is visualized as an image. A fixing method of using two fixing rolls, which is used in an image forming apparatus of using a developer liquid, is examined as a method of fixing the toner image on the recording medium.

### SUMMARY

According to an aspect of the invention, there is an image forming apparatus including:

an image holding member;

a charging unit that charges a surface of the image holding member;

an electrostatic charge image forming unit that forms an electrostatic charge image on a charged surface of the image holding member;

a developing unit that stores a developer containing a toner and develops the electrostatic charge image formed on a surface of the image holding member by using the developer so as to form a toner image;

a transfer unit that transfers the toner image formed on the surface of the image holding member onto a surface of a recording medium; and

a fixing unit that performs an operation of heating and pressing to the toner image on the recording medium twice or more by using one or more of a heating and pressing member which contacts with the toner image,

wherein the toner contains a binder resin, a colorant, and a release agent, and has a sea and island structure of a sea portion containing the binder resin and an island portion containing the release agent,

a maximum frequent value in distribution of the following eccentricity B of the island portion containing the release agent is in a range of from 0.75 to 0.95, and

a skewness in the distribution of the following eccentricity B is in a range of from -1.10 to -0.50,

the eccentricity B being represented by the following expression (1):

wherein D indicates an equivalent circle diameter ( $\mu\text{m}$ ) of the toner in an observation of a cross-section of the toner, and d indicates a distance ( $\mu\text{m}$ ) from the centroid of the toner to the centroid of the island portion containing the release agent in the observation of a cross-section of the toner.

### BRIEF DESCRIPTION OF THE DRAWINGS

Exemplary embodiments of the present invention will be described in detail based on the following figures, wherein:

FIG. 1 is a schematic configuration diagram illustrating an example of an image forming apparatus according to this exemplary embodiment;

FIG. 2 is a schematic diagram illustrating an example of a multi-stage fixing type fixing device according to this exemplary embodiment;

FIG. 3 is a schematic diagram illustrating a power feeding addition method; and

FIG. 4 is a diagram illustrating an example of distribution of eccentricity B of a release agent domain in a toner according to this exemplary embodiment.

### DETAILED DESCRIPTION

Hereinafter, an exemplary embodiment of the invention will be described in detail.

#### Image Forming Apparatus/Image Forming Method

An image forming apparatus according to this exemplary embodiment includes an image holding member, a charging unit, an electrostatic charge image forming unit, a developing unit, a transfer unit, and a fixing unit. The charging unit charges a surface of the image holding member. The electrostatic charge image forming unit forms an electrostatic charge image on the charged surface of the image holding member. The developing unit develops the electrostatic charge image formed on the surface of the image holding member by using an electrostatic charge image developing toner (also simply referred to as a "toner" below), so as to form a toner image. The transfer unit transfers the toner image formed on the surface of the image holding member onto a surface of a recording medium. The fixing unit fixes the toner image to the recording medium.

In this exemplary embodiment, the fixing unit (fixing process) fixes the toner image in such a manner that an operation of heating and pressing is performed on the toner image on the recording medium twice or more by using a heating and pressing member which contacts with the toner image.

In this exemplary embodiment, the developing unit stores an electrostatic charge image developing toner as the toner and the electrostatic charge image developing toner is used in a developing process. The electrostatic charge image developing toner contains a binder resin, a colorant, and a release agent. The electrostatic charge image developing toner has a sea and island structure in which a sea portion containing the binder resin and an island portion containing the release agent are provided. In the electrostatic charge image developing toner, a maximum frequent value in distribution of the following eccentricity B of the island portion containing the release agent is in a range of from 0.75 to 0.95, a skewness in the distribution of the following eccentricity B is in a range of from -1.10 to -0.50, and the eccentricity B is represented by the following expression (1):

wherein D indicates an equivalent circle diameter ( $\mu\text{m}$ ) of the toner in an observation of a cross-section of the toner, and d indicates a distance ( $\mu\text{m}$ ) from the centroid of the toner to the centroid of the island portion containing the release agent in the observation of a cross-section of the toner.

With the above configuration, the image forming apparatus and the image forming method according to this exemplary embodiment may also prevent adhering (offset) of the toner to the heating and pressing member in a multi-stage fixing method (method in which a toner image is fixed by performing an operation of heating and pressing twice or more). The reasons thereof are not clear, but presumed as follows.

In the fixing method in which fixing is performed by causing the heating and pressing member to contact with a toner image on a recording medium and performing the operation of heating and pressing, a state of bleeding of the release agent from the toner in heating and pressing matters in view of preventing adhering (offset) of the toner to the heating and pressing member.

Particularly, in the toner containing the binder resin deteriorated due to conditions of continuous exposure in a high temperature and high humidity environment for a long time, occurrence of the offset of the toner to the heating and pressing member is increased. Thus, bleeding of the release agent becomes more important. For this reason, a method is considered in which bleeding of the release agent from the toner in heating and pressing is improved and adhesion resistance (offset resistance) of the toner to the heating and pressing member is improved by using a toner in which the release agent unevenly exists only at a surface layer portion instead of a toner in which the release agent unevenly exists only in the inside.

Fixing is performed by using a fixing method (multi-stage fixing method) in which the heating and pressing member contacts with the toner image on the recording medium twice or more and the operation of heating and pressing is performed twice or more. Particularly, in view of improving gloss of an image, a multi-stage fixing method in which a first heating and pressing operation serves a fixing function, and a second heating and pressing operation serves a gloss improvement function is employed. For example, since as the thickness of a recording medium becomes thicker, improvement of gloss of an image becomes more difficult, an effect of improvement of gloss obtained by using the above-described multi-stage fixing method is shown more.

However, in a multi-stage fixing type image forming apparatus, when a toner in which the release agent unevenly exists only at the surface layer portion is used, offset of the toner to the heating and pressing member may occur in the second heating and pressing operation. In the first heating and pressing operation, the release agent which unevenly exists at the surface layer portion of the toner bleeds well and the release agent is interposed between the heating and pressing member and the toner image, and thus the occurrence of the offset of the toner is prevented. Since the release agent which unevenly exists only at the surface layer portion bleeds in the first heating and pressing operation, the second heating and pressing operation is performed in a state where a remaining amount of the release agent in the toner is small. That is, since an amount of bleeding of the release agent from the toner is relatively reduced in the second heating and pressing operation, an amount of the release agent interposed between the heating and pressing member and the toner image in the second operation is also reduced. In addition, a portion of the release agent which bleeds in the first operation adheres to the heating and pressing member,

as it is, in the first operation. However, when a cleaning member is disposed on a surface of the heating and pressing member, the adhered release agent is cleaned from the heating and pressing member and does not return to the toner image. From this point, the amount of the release agent between the heating and pressing member and the toner image in the second heating and pressing operation is further reduced. Thus, offset of the toner in the second heating and pressing operation appears to occur.

The toner for this exemplary embodiment will be described. The eccentricity B of the island portion containing the release agent (also referred to as a "release agent domain" below) in the specific toner is an index indicating a distance of the centroid of the release agent domain from the centroid of the toner. A larger value of the eccentricity B indicates that the release agent domain exists closer to the surface of the toner. A smaller value of the eccentricity B indicates that the release agent domain exists closer to the center of the toner. The maximum frequent value in the distribution of the eccentricity B indicates a portion at which the release agent domain exists in the largest amount in a radial direction of the toner. The skewness of the distribution of the eccentricity B indicates bilateral symmetry of the distribution. Specifically, the skewness of the distribution of the eccentricity B indicates a degree of unevenness from the maximum frequent value in the distribution. That is, the skewness of the distribution of the eccentricity B indicates a degree of the distribution of the release agent domain from the portion where the release agent domain exists in the largest amount in the diameter direction of the toner.

That is, the maximum frequent value in the distribution of the eccentricity B of the release agent domain being in a range of from 0.75 to 0.95 means that the release agent domain exists in the largest amount at a position close to a surface layer portion of the toner. The skewness of the distribution of the eccentricity B of the release agent domain being in a range of from -1.10 to -0.50 means that the release agent domain is distributed inwardly from the surface layer portion of the toner with a gradient (see FIG. 4).

In this manner, the toner in which the maximum frequent value and the skewness of the distribution of the eccentricity B of the release agent domain respectively satisfy the above-described ranges is a toner in which the release agent domain exists in the largest amount at the surface layer portion and is distributed so as to have a gradient from the inside of the toner toward the surface layer portion. In the toner according to this exemplary embodiment, the release agent exists in the largest amount at the surface layer portion and thus the release agent bleeds well from the surface layer portion in the first heating and pressing operation of the multi-stage fixing method, and the release agent is interposed between the heating and pressing member and the toner image so as to prevent the occurrence of the offset of the toner. In addition, the release agent exists with a gradient in the inside of the toner and thus the release agent which exists in the inside bleeds from the toner in the second heating and pressing operation and the release agent is interposed well between the heating and pressing member in the second heating and pressing operation, and the toner image. Accordingly, the occurrence of the offset of the toner in the second heating and pressing operation is further prevented.

In this manner, in this exemplary embodiment, it is presumed that adhering (offset) of the toner to the heating and pressing member is also prevented in the multi-stage fixing method.

In one toner of the related art, the release agent is positioned so as to be in the vicinity of a surface by using a difference in hydrophilic-hydrophobic properties between a binder resin and a release agent which are dissolved in a solvent. In the other toner of the related art, a release agent is positioned so as to be in the vicinity of a surface by using kneading and pulverizing method with an uneven distribution control resin, and the uneven distribution control resin has both of a portion close to a polarity of a binder resin and a portion close to a polarity of the release agent. However, all of the toners control a position of a release agent in a toner by using a physical property of a material and do not cause distribution of the release agent domain of a toner to have a gradient.

In this exemplary embodiment, the multi-stage fixing method (method in which a toner image is fixed by performing an operation of heating and pressing twice or more) may have a configuration in which two or more heating and pressing members are provided, and a recording medium passes through each of the plural heating and pressing members once, or may have a configuration in which one heating and pressing member is provided, and a recording medium repeatedly passes through the heating and pressing member twice or more. However, in view of more improving gloss of an image, the configuration in which two or more heating and pressing members are provided, and a recording medium passes through each of the plural heating and pressing members once is more preferable.

The image forming apparatus and the image forming method according to this exemplary embodiment will be described below in detail.

#### Electrostatic Charge Image Developing Toner

First, in this exemplary embodiment, a toner which is stored in a developing device and is used in the developing process will be described in detail.

The toner in this exemplary embodiment has the sea and island structure in which the sea portion containing the binder resin and the island portion containing the release agent are provided. That is, the toner has the sea and island structure in which the release agent exists in a continuous phase of the binder resin so as to have an island shape. The release agent domain, preferably, may not exist at the center portion (centroid portion) of the toner in observation of a cross-section of the toner, from a viewpoint of prevention of separation deficiency and prevention of uneven gloss.

In the toner having the sea and island structure, the maximum frequent value in the distribution of the eccentricity B of the release agent domain (island portion containing the release agent) is in a range of from 0.75 to 0.95, and, from the viewpoint of prevention of the occurrence of adhering (offset) of the toner in the multi-stage fixing method, is preferably in a range of from 0.80 to 0.95, more preferably in a range of from 0.80 to 0.90, and most preferably in a range of from 0.85 to 0.90.

The skewness in the distribution of the eccentricity B of the release agent domain (island portion containing the release agent) is in a range of from -1.10 to -0.50, preferably in a range of from -0.60 to -0.40 from a viewpoint of prevention of the occurrence of adhering (offset) of the toner in the multi-stage fixing method, and more preferably in a range of from -0.95 to -0.65.

The kurtosis in the distribution of the eccentricity B of the release agent domain (island portion containing the release agent) is preferably in a range of from -0.20 to +1.50, more preferably in a range of from -0.15 to +1.40, further preferably in a range of from -0.10 to +1.40, and most preferably in a range of from -0.10 to +1.30, from a

viewpoint of prevention of the occurrence of adhering (offset) of the toner in the multi-stage fixing method.

The kurtosis is an index indicating a sharp point of a vertex (that is, the maximum frequent value in the distribution) in the distribution of the eccentricity B. The kurtosis being in the above range indicates a state where an apex portion (maximum frequent value) is not excessively sharp in the distribution of the eccentricity B and the distribution having an apex portion which is appropriately curved while being sharp is made. For this reason, it is a state where the release agent exists on the surface and exists appropriately in an inward direction in the toner, and thus adhering (offset) of the toner in the multi-stage fixing method is further prevented.

15 A confirming method of the sea and island structure of the toner will be described.

The sea and island structure of the toner is confirmed, for example, by a method of observing a cross-section of the toner (toner particle) using a transmission electron microscope, or a method of dyeing a cross-section of the toner particle with ruthenium tetroxide and observing the dyed cross-section using a scanning electron microscope. The method of observation using a scanning electron microscope is preferable in that the release agent domain in the cross-section of the toner may be observed more clearly. As the scanning electron microscope, a model which has been known well to those skilled in the related art may be used. For example, SU8020 manufactured by Hitachi High-Technologies Corporation, JSM-7500F manufactured by JEOL Ltd., and the like are included.

35 Specifically, an observing method is performed as follows. First, a toner (toner particle) to be measured is embedded in an epoxy resin, and then the epoxy resin is cured. This cured substance is cut into a thin section with a microtome including a diamond blade to thereby obtain an observation sample in which a cross-section of the toner is exposed. Dyeing with ruthenium tetroxide is performed on the thin observation sample and the cross-section of the toner is observed by using a scanning electron microscope. 40 Using this observing method, a sea and island structure in which a release agent having a brightness difference (contrast) caused by a dyeing degree with respect to a continuous phase of a binder resin exists so as to have an island shape in the cross-section of the toner is observed.

45 Next, a measuring method of the eccentricity B of the release agent domain will be described.

The eccentricity B of the release agent domain is measured as follows. First, an image is recorded at magnification which allows a cross-section of one toner (toner particle) to come in sight, by using the confirming method of the sea and island structure. Image analysis for the recorded image is performed under a condition of  $0.010000 \mu\text{m}/\text{pixel}$  by using image analysis software (WINROOF manufactured by MITANI Corporation). A shape of the cross-section of the toner is extracted by this image analysis by using a brightness difference (contrast) between the epoxy resin used in embedding and the binder resin of the toner. A projected area is obtained based on the extracted shape of the cross-section of the toner. An equivalent circle diameter is obtained from the projected area. The equivalent circle diameter is calculated by an expression of  $2\sqrt{(\text{projected area}/\pi)}$ . The obtained equivalent circle diameter is set as an equivalent circle diameter D of the toner in observation of the cross-section of the toner.

65 A centroid position is obtained based on the extracted shape of the cross-section of the toner. Subsequently, a shape of the release agent domain is extracted by using a bright-

ness difference (contrast) between the binder resin and the release agent, and a centroid position of the release agent domain is obtained. Each of the centroid positions is obtained as follows. x coordinates of the centroids are values obtained by dividing summation of  $x_i$  coordinate values by n, and y coordinates of the centroids are values obtained by dividing summation of  $y_i$  coordinate values by n, when the number of pixels in an area of the extracted toner or the extracted release agent domain is set as n, xy coordinates of each pixel are set as  $x_i$  and  $y_i$  ( $i=1, 2, \dots, n$ ). A distance between the centroid position of the cross-section of the toner and the centroid position of the release agent domain is obtained. The obtained distance is set as a distance d from the centroid of the toner to the centroid of the island portion containing the release agent in observation of the cross-section of the toner.

At last, the eccentricity B of the release agent domain is obtained based on each of the equivalent circle diameter D and the distance d by using Expression (1) (eccentricity  $B=2d/D$ ). Similarly, the above-described operation is performed on each of plural release agent domains in the cross-section of one toner (toner particle) and thereby the eccentricity B of the release agent domain is obtained.

Next, a calculating method of the maximum frequent value in distribution of the eccentricity B of the release agent domain will be described.

First, the eccentricity B of the release agent domain for 200 toners (toner particles) is measured as described above. Data of the obtained eccentricity B of each of the release agent domains is subjected to statistical analysis processing in a data sections from 0 in increment of 0.01, and thereby the distribution of the eccentricity B is obtained. The maximum frequent value in the obtained distribution, that is, a value of a data section which appears most in the distribution of the eccentricity B of the release agent domain is obtained. The value of this data section is set as the maximum frequent value in the distribution of the eccentricity B of the release agent domain.

Next, a calculating method of the skewness in the distribution of the eccentricity B of the release agent domain will be described.

First, the distribution of the eccentricity B of the release agent domain is obtained as described above. The skewness in the distribution of the eccentricity B is obtained based on the following expression. In the following expression, the skewness is set as  $Sk$ , the number of pieces of data of the eccentricity B of the release agent domain is set as n, values of data of the eccentricity B of the respective release agent domains are set as  $x_i$  ( $i=1, 2, \dots, n$ ), an average value of all pieces of data of the eccentricity B of the release agent domain is set as  $x$  ( $x$  with a bar above), and a standard deviation of all pieces of data of the eccentricity B of the release agent domain is set as s.

$$Sk = \frac{n}{(n-1)(n-2)} \sum_{i=1}^n \left( \frac{x_i - \bar{x}}{s} \right)^3$$

Next, a calculating method of the kurtosis in the distribution of the eccentricity B of the release agent domain will be described.

First, the distribution of the eccentricity B of the release agent domain is obtained as described above. The kurtosis in the obtained distribution of the eccentricity B is obtained based on the following expression. In the following expres-

sion, the kurtosis is set as  $Ku$ , the number of pieces of data of the eccentricity B of the release agent domain is set as n, values of data of the eccentricity B of the respective release agent domains are set as  $x_i$  ( $i=1, 2, \dots, n$ ), an average value of all pieces of data of the eccentricity B of the release agent domain is set as  $x$  ( $x$  with a bar above), and a standard deviation of all pieces of data of the eccentricity B of the release agent domain is set as s.

$$Ku = \frac{n(n+1)}{(n-1)(n-2)(n-3)} \sum_{i=1}^n \left( \frac{x_i - \bar{x}}{s} \right)^4 - \frac{3(n-1)^2}{(n-2)(n-3)}$$

Regarding a method for satisfying distribution characteristics of the eccentricity B of the release agent domain in a toner, it will be described in a method of preparing the toner.

Components of the specific toner will be described below. The specific toner contains a binder resin, a colorant, and a release agent. Specifically, the toner contains toner particles including the binder resin, the colorant, and the release agent. The toner may contain an external additive adhering to a surface of the toner particle.

#### Release Agent

Examples of the release agent include hydrocarbon waxes; natural waxes such as carnauba wax, rice wax, and candelilla wax; synthetic or mineral/petroleum waxes such as montan wax; and ester waxes such as fatty acid esters and montanic acid esters; and the like. The release agent is not limited to these examples.

Among these substances, as the release agent, the hydrocarbon wax (waxes having hydrocarbon as a skeleton) is preferable. The hydrocarbon wax is appropriate because the release agent domain is easily formed and rapid bleeding to the surface of the toner (toner particle) easily occurs in fixing.

A melting temperature of the release agent is preferably in a range from 50°C. to 110°C., and more preferably in a range from 60°C. to 100°C.

The melting temperature is obtained from a DSC curve obtained by differential scanning calorimetry (DSC). More specifically, the melting temperature is obtained from "Melting Peak Temperature" described in the method of obtaining a melting temperature in JIS K 7121-1987 "Testing Methods for Transition Temperatures of Plastics".

The content of the release agent is, for example, preferably in a range of from 1% by weight to 20% by weight, and more preferably in a range of from 5% by weight to 15% by weight relative to the entire toner particles.

#### Binder Resin

Examples of the binder resin include vinyl resins formed of homopolymers of monomers such as styrenes (for example, styrene, parachlorostyrene, and  $\alpha$ -methylstyrene), (meth)acrylates (for example, methyl acrylate, ethyl acrylate, n-propyl acrylate, n-butyl acrylate, lauryl acrylate, 2-ethylhexyl acrylate, methyl methacrylate, ethyl methacrylate, n-propyl methacrylate, laurylmethacrylate, and 2-ethylhexyl methacrylate), ethylenically unsaturated nitriles (for example, acrylonitrile and methacrylonitrile), vinyl ethers (for example, vinyl methyl ether and vinyl isobutyl ether), vinyl ketones (for example, vinyl methyl ketone, vinyl ethyl ketone, and vinyl isopropenyl ketone), and olefins (for example, ethylene, propylene, and butadiene), or copolymers obtained by combining two or more kinds of these monomers.

Examples of the binder resin also include a non-vinyl resin such as an epoxy resin, a polyester resin, a polyurethane resin, a polyamide resin, a cellulose resin, a polyether resin, and modified rosin, mixtures thereof with the above-described vinyl resin, or graft polymer obtained by polymerizing a vinyl monomer with the coexistence of such non-vinyl resins.

These binder resins may be used singly or in combination of two or more kinds thereof.

As the binder resin, a polyester resin is appropriate.

As the polyester resin, for example, a well-known polyester resin is included.

Examples of the polyester resin include condensation polymers of polyvalent carboxylic acids and polyols. A commercially available product or a synthesized product may be used as the polyester resin.

Examples of the polyvalent carboxylic acid include aliphatic dicarboxylic acids (for example, oxalic acid, malonic acid, maleic acid, fumaric acid, citraconic acid, itaconic acid, glutaconic acid, succinic acid, alkenyl succinic acid, adipic acid, and sebatic acid), alicyclic dicarboxylic acids (for example, cyclohexanedicarboxylic acid), aromatic dicarboxylic acids (for example, terephthalic acid, isophthalic acid, phthalic acid, and naphthalenedicarboxylic acid), anhydrides thereof, or lower alkyl esters (having, for example, from 1 to 5 carbon atoms) thereof. Among these substances, for example, aromatic dicarboxylic acids are preferably used as the polyvalent carboxylic acid.

As the polyvalent carboxylic acid, a tri- or higher-valent carboxylic acid employing a crosslinked structure or a branched structure may be used in combination with a dicarboxylic acid. Examples of the tri- or higher-valent carboxylic acid include trimellitic acid, pyromellitic acid, anhydrides thereof, or lower alkyl esters (having, for example, from 1 to 5 carbon atoms) thereof.

The polyvalent carboxylic acids may be used singly or in combination of two or more types thereof.

Examples of the polyol include aliphatic diols (for example, ethylene glycol, diethylene glycol, triethylene glycol, propylene glycol, butanediol, hexanediol, and neopentyl glycol), alicyclic diols (for example, cyclohexanediol, cyclohexanedimethanol, and hydrogenated bisphenol A), and aromatic diols (for example, ethylene oxide adduct of bisphenol A and propylene oxide adduct of bisphenol A). Among these, for example, aromatic diols and alicyclic diols are preferably used, and aromatic diols are more preferably used as the polyol.

As the polyol, a tri- or higher-valent polyol employing a crosslinked structure or a branched structure may be used in combination together with diol. Examples of the tri- or higher-valent polyol include glycerin, trimethylolpropane, and pentaerythritol.

The polyol may be used singly or in combination of two or more types thereof.

The glass transition temperature (Tg) of the polyester resin is preferably from 50°C. to 80°C., and more preferably from 50°C. to 65°C.

The glass transition temperature is obtained by a DSC curve which is obtained by a differential scanning calorimetry (DSC), and more specifically, is obtained by "Extrapolating Glass Transition Starting Temperature" disclosed in a method for obtaining the glass transition temperature of "Testing Methods for Transition Temperatures of Plastics" in JIS K-7121-1987.

The weight-average molecular weight (Mw) of the polyester resin is preferably in a range from 5,000 to 1,000,000, and more preferably in a range from 7,000 to 500,000.

The number-average molecular weight (Mn) of the polyester resin is preferably in a range from 2,000 to 100,000.

A molecular weight distribution Mw/Mn of the polyester resin is preferably in a range from 1.5 to 100, and more preferably in a range from 2 to 60.

The weight-average molecular weight and the number-average molecular weight are measured by using gel permeation chromatography (GPC). Molecular weight measurement by using GPC is performed by using •HLC-8120GPC (GPC manufactured by TOSOH Corporation) as a measurement device, by using TSKGEL SUPERHM-M (15 cm) (column manufactured by TOSOH Corporation), and by using a THF solvent. The weight-average molecular weight and the number-average molecular weight are calculated by using a molecular weight calibration curve which is created based on this measurement result by using a monodisperse polystyrene standard sample.

The polyester resin is obtained by a known preparing method. Specific examples thereof include a method of performing a reaction at a polymerization temperature set to be in a range of from 180°C. to 230°C., if necessary, under reduced pressure in the reaction system, while removing water or an alcohol generated during condensation.

When monomers of the raw materials are not dissolved or compatibilized under a reaction temperature, a high-boiling-point solvent may be added as a solubilizing agent to dissolve the monomers. In this case, a polycondensation reaction is performed while distilling away the solubilizing agent. When a monomer having poor compatibility is present in a copolymerization reaction, the monomer having poor compatibility and an acid or an alcohol to be polycondensed with the monomer may be previously condensed and then polycondensed with the major component.

The content of the binder resin is, for example, preferably in a range of from 40% by weight to 95% by weight, more preferably in a range of from 50% by weight to 90% by weight, and further preferably in a range of from 60% by weight to 85% by weight relative to the entire toner particles.

#### Colorant

Examples of the colorant include various pigments such as carbon black, chrome yellow, Hansa yellow, benzidine yellow, threne yellow, quinoline yellow, pigment yellow, permanent orange GTR, pyrazolone orange, vulcan orange, watchung red, permanent red, brilliant carmine 3B, brilliant carmine 6B, DuPont oil red, pyrazolone red, lithol red, Rhodamine B Lake, Lake Red C, pigment red, rose bengal, aniline blue, ultramarine blue, calco oil blue, methylene blue chloride, phthalocyanine blue, pigment blue, phthalocyanine green, and malachite green oxalate, and various dyes such as acridine dyes, xanthene dyes, azo dyes, benzoquinone dyes, azine dyes, anthraquinone dyes, thioindigo dyes, dioxadine dyes, thiazine dyes, azomethine dyes, indigo dyes, phthalocyanine dyes, aniline black dyes, polymethine dyes, triphenylmethane dyes, diphenylmethane dyes, and thiazole dyes.

The colorant may be used singly or in combination of two or more types thereof.

If necessary, the colorant may be surface-treated or used in combination with a dispersing agent. Plural types of colorants may be used in combination.

The content of the colorant is, for example, preferably in a range of from 1% by weight to 30% by weight, and more preferably in a range of from 3% by weight to 15% by weight relative to the entire toner particles.

## Other Additives

Examples of other additives include known additives such as a magnetic material, a charge-controlling agent, and inorganic powder. The toner particles contain these additives as internal additives.

## Characteristics of Toner Particles

The toner particles may be toner particles having a single-layer structure, or be toner particles having a so-called core/shell structure composed of a core (core particle) and a coating layer (shell layer) coated on the core.

Here, toner particles having a core/shell structure is preferably composed of, for example, a core containing a binder resin, and other additives such as a colorant and a release agent and a coating layer containing a binder resin.

The volume average particle diameter (D50v) of the toner particles is preferably in a range of from 2  $\mu\text{m}$  to 10  $\mu\text{m}$ , and more preferably in a range of from 4  $\mu\text{m}$  to 8  $\mu\text{m}$ .

Various average particle diameters and various particle size distribution indices of the toner particles are measured by using a COULTER MULTISIZER II (manufactured by Beckman Coulter, Inc.) and ISOTON-II (manufactured by Beckman Coulter, Inc.) as an electrolyte.

In the measurement, from 0.5 mg to 50 mg of a measurement sample is added to 2 ml of a 5% aqueous solution of surfactant (preferably sodium alkylbenzene sulfonate) as a dispersing agent. The obtained material is added to from 100 ml to 150 ml of the electrolyte.

The electrolyte in which the sample is suspended is subjected to a dispersion treatment using an ultrasonic disperser for 1 minute, and a particle size distribution of particles having a particle diameter of from 2  $\mu\text{m}$  to 60  $\mu\text{m}$  is measured by a COULTER MULTISIZER II using an aperture having an aperture diameter of 100  $\mu\text{m}$ . 50,000 particles are sampled.

Cumulative distributions by volume and by number are drawn from the side of the smallest diameter with respect to particle size ranges (channels) separated based on the measured particle size distribution. The particle diameter when the cumulative percentage becomes 16% is defined as that corresponding to a volume average particle diameter D16v and a number average particle diameter D16p, while the particle diameter when the cumulative percentage becomes 50% is defined as that corresponding to a volume average particle diameter D50v and a number average particle diameter D50p. Furthermore, the particle diameter when the cumulative percentage becomes 84% is defined as that corresponding to a volume average particle diameter D84v and a number average particle diameter D84p.

Using these, a volume average particle size distribution index (GSDv) is calculated as  $(D84v/D16v)^{1/2}$ , while a number average particle size distribution index (GSDp) is calculated as  $(D84p/D16p)^{1/2}$ .

The shape factor SF1 of the toner particles is preferably from 110 to 150, and more preferably from 120 to 140.

The shape factor SF1 is obtained through the following expression.

$$SF1 = (ML^2/4) \times (\pi/4) \times 100$$

Expression:

In the foregoing expression, ML represents an absolute maximum length of a toner, and A represents a projected area of a toner.

Specifically, the shape factor SF1 is numerically converted mainly by analyzing a microscopic image or a scanning electron microscopic (SEM) image by using of an image analyzer, and is calculated as follows. That is, an optical microscopic image of particles scattered on a surface of a glass slide is input to an image analyzer LUZEX

through a video camera to obtain maximum lengths and projected areas of 100 particles, values of SF1 are calculated through the foregoing expression, and an average value thereof is obtained.

## 5 External Additive

Examples of the external additive include inorganic particles. Examples of the inorganic particles include  $\text{SiO}_2$ ,  $\text{TiO}_2$ ,  $\text{Al}_2\text{O}_3$ ,  $\text{CuO}$ ,  $\text{ZnO}$ ,  $\text{SnO}_2$ ,  $\text{CeO}_2$ ,  $\text{Fe}_2\text{O}_3$ ,  $\text{MgO}$ ,  $\text{BaO}$ ,  $\text{CaO}$ ,  $\text{K}_2\text{O}$ ,  $\text{Na}_2\text{O}$ ,  $\text{ZrO}_2$ ,  $\text{CaO} \cdot \text{SiO}_2$ ,  $\text{K}_2\text{O} \cdot (\text{TiO}_2)_n$ ,  $\text{Al}_2\text{O}_3 \cdot 2\text{SiO}_2$ ,  $\text{CaCO}_3$ ,  $\text{MgCO}_3$ ,  $\text{BaSO}_4$ , and  $\text{MgSO}_4$ .

Surfaces of the inorganic particles as an external additive are preferably subjected to a hydrophobizing treatment with a hydrophobizing agent. The treatment with a hydrophobizing agent is performed by, for example, dipping the inorganic particles in a hydrophobizing agent. The hydrophobizing agent is not particularly limited and examples thereof include a silane coupling agent, silicone oil, a titanate coupling agent, and an aluminum coupling agent. These may be used singly or in combination of two or more kinds thereof.

Generally, the amount of the hydrophobizing agent is, for example, from 1 part by weight to 10 parts by weight with respect to 100 parts by weight of the inorganic particles.

Examples of the external additive also include resin particles (resin particles such as polystyrene, polymethyl methacrylate (PMMA), and melamine resin particles) and a cleaning aid (for example, metal salt of higher fatty acid represented by zinc stearate, and fluorine polymer particles).

The amount of the external additive externally added is, for example, preferably in a range of from 0.01% by weight to 5% by weight, and more preferably in a range of from 0.01% by weight to 2.0% by weight relative to the toner particles.

## Method of Preparing Toner

35 Next, a method of preparing the toner will be described. The toner is obtained by externally adding an external additive to toner particles after preparing the toner particles.

The toner particles may be prepared using any of a dry preparing method (for example, kneading and pulverizing method) and a wet preparing method (for example, aggregation and coalescence method, suspension and polymerization method, and dissolution and suspension method). The toner particle preparing method is not particularly limited to these preparing methods, and a known preparing method is employed.

45 Among these methods, the toner particles may preferably be obtained by the aggregation and coalescence method.

For preparing the toner (toner particle) which satisfies the above-described distribution characteristics of the eccentricity B of the release agent domain as described above, the toner particle may preferably be prepared by an aggregation and coalescence method described below.

Specifically, the toner particle is preferably prepared by processes as follows: a process of preparing each dispersion (dispersion preparation process); a process (first aggregated particle forming process); a process (second aggregated particle forming process); and a process (coalescence process). In the first aggregated particle forming process, particles are aggregated in a dispersion obtained by mixing a first resin particle dispersion and a colorant particle dispersion, and thereby first aggregated particles are formed. The first resin particle dispersion is obtained by dispersing first resin particles corresponding to the binder resin, and the colorant particle dispersion is obtained by dispersing particles of the colorant (also referred to as "colorant particles" below). In the second aggregated particle forming process, a dispersion mixture in which second resin particles corre-

sponding to the binder resin and particles of the release agent (also referred to as “release agent particles” below) are dispersed is prepared. After a first aggregated particle dispersion in which the first aggregated particles are dispersed is prepared, the dispersion mixture is sequentially added to the first aggregated particle dispersion while the concentration of the release agent particles in the dispersion mixture gradually increases. Thus, the second resin particles and the release agent particles are aggregated on a surface of the first aggregated particles, and thereby second aggregated particles are formed. In the coalescence process, a second aggregated particle dispersion in which the second aggregated particles are dispersed is heated to coalesce the second aggregated particles, and thereby toner particles are formed.

The method of preparing the toner particle is not limited to the above descriptions. For example, particles are aggregated in a dispersion mixture obtained by mixing the resin particle dispersion and the colorant particle dispersion. Then, a release agent particle dispersion is added to the dispersion mixture in the process of aggregation while increasing an addition speed gradually or while increasing the concentration of the release agent particles increases. Thus, aggregation of particles proceeds more, and thereby aggregated particles are formed. The toner particles may be formed by coalescing the aggregated particles.

The processes will be described below in detail.

#### Preparation Process of Dispersion

First, respective dispersions are prepared by using an aggregation and coalescence method. Specifically, a first resin particle dispersion in which first resin particles corresponding to the binder resin are dispersed, a colorant particle dispersion in which colorant particles are dispersed, a second resin particle dispersion in which second resin particles corresponding to the binder resin are dispersed, and a release agent particle dispersion in which release agent particles are dispersed are prepared.

In the dispersion preparation process, descriptions will be made, referring the first resin particles and the second resin particles to as “resin particles” collectively.

The resin particle dispersion is prepared by, for example, dispersing resin particles in a dispersion medium using a surfactant.

Examples of the dispersion medium used for the resin particle dispersion include aqueous mediums.

Examples of the aqueous mediums include water such as distilled water and ion exchange water, and alcohols. These may be used singly or in combination of two or more kinds thereof.

Examples of the surfactant include anionic surfactants such as a sulfuric ester salt, a sulfonate, a phosphate ester, and a soap; cationic surfactants such as an amine salt and a quaternary ammonium salt; and nonionic surfactants such as polyethylene glycol, an ethylene oxide adduct of alkyl phenol, and polyol. Among these, anionic surfactants and cationic surfactants are particularly preferably used. Non-ionic surfactants may be used in combination with anionic surfactants or cationic surfactants.

The surfactants may be used singly or in combination of two or more kinds thereof.

Regarding the resin particle dispersion, as a method of dispersing the resin particles in the dispersion medium, a common dispersing method using, for example, a rotary shearing-type homogenizer, or a ball mill, a sand mill, or a DYNOMILL having media is exemplified. Depending on the kind of the resin particles, resin particles may be dispersed in the resin particle dispersion according to, for example, a phase inversion emulsification method.

The phase inversion emulsification method includes: dissolving a resin to be dispersed in a hydrophobic organic solvent in which the resin is soluble; conducting neutralization by adding an abase to an organic continuous phase (O phase); and converting the resin (so-called phase inversion) from W/O to O/W by putting an aqueous medium (W phase) to form a discontinuous phase, thereby dispersing the resin as particles in the aqueous medium.

A volume average particle diameter of the resin particles dispersed in the resin particle dispersion is, for example, preferably from 0.01  $\mu\text{m}$  to 1  $\mu\text{m}$ , more preferably from 0.08  $\mu\text{m}$  to 0.8  $\mu\text{m}$ , and even more preferably from 0.1  $\mu\text{m}$  to 0.6  $\mu\text{m}$ .

Regarding the volume average particle diameter of the resin particles, a cumulative distribution by volume is drawn from the side of the smallest diameter with respect to particle size ranges (channels) separated using the particle size distribution obtained by the measurement with a laser diffraction-type particle size distribution measuring device (for example, LA-700 manufactured by Horiba, Ltd.), and a particle diameter when the cumulative percentage becomes 50% with respect to the entire particles is measured as a volume average particle diameter D50v. The volume average particle diameter of the particles in other dispersions is also measured in the same manner.

The content of the resin particles contained in the resin particle dispersion is, for example, preferably from 5% by weight to 50% by weight, and more preferably from 10% by weight to 40% by weight.

For example, the colorant particle dispersion and the release agent particle dispersion are also prepared in the same manner as in the case of the resin particle dispersion. That is, the particles in the resin particle dispersion are the same as the colorant particles dispersed in the colorant particle dispersion and the release agent particles dispersed in the release agent particle dispersion, in terms of the volume average particle diameter, the dispersion medium, the dispersing method, and the content of the particles.

#### First Aggregated Particle Forming Process

Next, the first resin particle dispersion and the colorant particle dispersion are mixed together.

The first resin particles and the colorant particles are heterogeneously aggregated in the dispersion mixture, and thereby first aggregated particles including first resin particles and colorant particles are formed.

Specifically, for example, an aggregating agent is added to the dispersion mixture and a pH of the dispersion mixture is adjusted to be acidic (for example, the pH is from 2 to 5). If necessary, a dispersion stabilizer is added. Then, the dispersion mixture is heated at the glass transition temperature of the first resin particles (specifically, for example, from a temperature 30° C. lower than the glass transition temperature of the first resin particles to a temperature 10° C. lower than the glass transition temperature thereof) to aggregate the particles dispersed in the dispersion mixture, and thereby the first aggregated particles are formed.

In the first aggregated particle forming process, for example, the aggregating agent may be added at room temperature (for example, 25° C.) under stirring of the dispersion mixture using a rotary shearing-type homogenizer, the pH of the dispersion mixture may be adjusted to be acidic (for example, the pH is from 2 to 5), a dispersion stabilizer may be added if necessary, and then the heating may be performed.

Examples of the aggregating agent include a surfactant having an opposite polarity to the polarity of the surfactant used as the dispersing agent to be added to the mixed

dispersion, an inorganic metal salt, and a bi- or higher-valent metal complex. Particularly, when a metal complex is used as the aggregating agent, the amount of the surfactant used is reduced and charging characteristics are improved.

If necessary, an additive may be used which forms a complex or a similar bond with the metal ions of the aggregating agent. A chelating agent is preferably used as the additive.

Examples of the inorganic metal salt include a metal salt such as calcium chloride, calcium nitrate, barium chloride, magnesium chloride, zinc chloride, aluminum chloride, and aluminum sulfate, and inorganic metal salt polymer such as polyaluminum chloride, polyaluminum hydroxide, and calcium polysulfide.

A water-soluble chelating agent may be used as the chelating agent. Examples of the chelating agent include oxycarboxylic acids such as tartaric acid, citric acid, and gluconic acid, iminodiacetic acid (IDA), nitrilotriacetic acid (NTA), and ethylenediaminetetraacetic acid (EDTA).

An addition amount of the chelating agent is, for example, preferably in a range of from 0.01 parts by weight to 5.0 parts by weight, and more preferably in a range of from 0.1 parts by weight to less than 3.0 parts by weight relative to 100 parts by weight of the first resin particles.

#### Second Aggregated Particle Forming Process

Next, after the first aggregated particle dispersion in which the first aggregated particles are dispersed is obtained, a dispersion mixture in which the second resin particles and the release agent particles are dispersed is sequentially added to the first aggregated particle dispersion while increasing the concentration of the release agent particles in the dispersion mixture gradually.

The second resin particles may be the same type as or a different type or from the first resin particles.

The second resin particles and the release agent particles are aggregated on surfaces of the first aggregated particles in a dispersion in which the first aggregated particles, the second resin particles, and the release agent particles are dispersed. Specifically, for example, in the first aggregated particle forming process, when a particle diameter of the first aggregated particle reaches a desired particle diameter, a dispersion mixture in which the second resin particles and the release agent particles are dispersed is added to the first aggregated particle dispersion while increasing the concentration of the release agent particles gradually. The dispersion is heated at a temperature which is equal to or less than the glass transition temperature of the second resin particles.

For example, the pH of the dispersion is substantially in a range of from 6.5 to 8.5, and thus the progress of the aggregation is stopped.

Aggregated particles in which the second resin particles and the release agent particles are attached to the surfaces of the first aggregated particles are formed through this process. That is, second aggregated particles in which aggregates of the second resin particles and the release agent particles are attached to the surfaces of the first aggregated particles are formed. At this time, since the dispersion mixture in which the second resin particles and the release agent particles are dispersed is sequentially added to the first aggregated particle dispersion while increasing the concentration of the release agent particles in the dispersion mixture gradually, the concentration (abundance ratio) of the release agent particles becomes gradually larger toward the radially outside direction of the particles, and the aggregates of the second resin particles and the release agent particles are attached to the surface of the first aggregated particle.

As a method of adding the dispersion mixture, a power feeding addition method may preferably be used. The dispersion mixture may be added to the first aggregated particle dispersion, with a gradual increase of the concentration of the release agent particles in the dispersion mixture, by using the power feeding addition method.

The method of adding the dispersion mixture using the power feeding addition method will be described with reference to the drawing.

FIG. 3 illustrates an apparatus used in the power feeding addition method. In FIG. 3, the reference numeral 311 indicates the first aggregated particle dispersion, the reference numeral 312 indicates the second resin particle dispersion, the reference numeral 313 indicates the release agent particle dispersion.

The apparatus illustrated in FIG. 3 includes a first storage tank 321, a second storage tank 322, and a third storage tank 323. In the first storage tank 321, the first aggregated particle dispersion in which the first aggregated particles are dispersed is stored. In the second storage tank 322, the second resin particle dispersion in which the second resin particles are dispersed is stored. In the third storage tank 323, the release agent particle dispersion in which the release agent particles are dispersed is stored.

The first storage tank 321 and the second storage tank 322 are linked to each other by using a first liquid transport tube 331. A first liquid transport pump 341 is provided in the middle of a path of the first liquid transport tube 331. Driving of the first liquid transport pump 341 causes the dispersion stored in the second storage tank 322 to be transported to the dispersion stored in the first storage tank 321 through the first liquid transport tube 331.

A first stirring apparatus 351 is disposed in the first storage tank 321. When driving of the first stirring apparatus 351 causes the dispersion stored in the second storage tank 322 to be transported to the dispersion stored in the first storage tank 321, the dispersions in the first storage tank 321 are stirred and mixed.

The second storage tank 322 and the third storage tank 323 are linked to each other by using a second liquid transport tube 332. A second liquid transport pump 342 is provided in the middle of a path of the second liquid transport tube 332. Driving of the second liquid transport pump 342 causes the dispersion stored in the third storage tank 323 to be transported to the dispersion stored in the second storage tank 322 through the second liquid transport tube 332.

A second stirring apparatus 352 is disposed in the second storage tank 322. When driving of the second stirring apparatus 352 causes the dispersion stored in the third storage tank 323 to be transported to the dispersion stored in the second storage tank 322, the dispersions in the second storage tank 322 are stirred and mixed.

In the apparatus illustrated in FIG. 3, first, the first aggregated particle forming process is performed and thereby a first aggregated particle dispersion is prepared, in the first storage tank 321. The first aggregated particle dispersion is stored in the first storage tank 321. The first aggregated particle forming process may be performed and thereby the first aggregated particle dispersion may be prepared in another tank, and then, the first aggregated particle dispersion may be stored in the first storage tank 321.

In this state, the first liquid transport pump 341 and the second liquid transport pump 342 are driven. This driving causes the second resin particle dispersion stored in the second storage tank 322 to be transported to the first

aggregated particle dispersion stored in the first storage tank 321. Driving of the first stirring apparatus 351 causes the dispersions in the first storage tank 321 to be stirred and mixed.

The release agent particle dispersion stored in the third storage tank 323 is transported to the second resin particle dispersion stored in the second storage tank 322. Driving of the second stirring apparatus 352 causes the dispersions in the second storage tank 322 to be stirred and mixed.

At this time, the release agent particle dispersion is sequentially transported to the second resin particle dispersion stored in the second storage tank 322, and thus the concentration of the release agent particles becomes higher gradually. For this reason, the dispersion mixture in which second resin particles and the release agent particles are dispersed is stored in the second storage tank 322, and this dispersion mixture is transported to the first aggregated particle dispersion stored in the first storage tank 321. The dispersion mixture is continuously transported with an increase of the concentration of the release agent particle dispersion in the dispersion mixture.

In this manner, the dispersion mixture in which the second resin particles and the release agent particles are dispersed may be added to the first aggregated particle dispersion with a gradual increase of the concentration of the release agent particles, by using the power feeding addition method.

In the power feeding addition method, the distribution characteristics of the release agent domain of the toner are adjusted by adjusting liquid transport starting time and a liquid transport speed for each of the dispersions which are respectively stored in the second storage tank 322 and the third storage tank 323. In the power feeding addition method, also by adjusting the liquid transport speed in the process of transporting of the dispersions respectively stored in the second storage tank 322 and the third storage tank 323, the distribution characteristics of the release agent domain of the toner are adjusted.

Specifically, for example, the maximum frequent value in the distribution of the eccentricity B of the release agent domain is adjusted depending on a period of time when transporting of the release agent particle dispersion to the second storage tank 322 from the third storage tank 323 is ended. More specifically, for example, if transporting of the release agent particle dispersion to the second storage tank 322 from the third storage tank 323 is ended before liquid transporting to the first storage tank 321 from the second storage tank 322 is ended, the concentration of the release agent particles in the dispersion mixture of the second storage tank 322 does not increase from that point of time. Thus, the maximum frequent value in the distribution of the eccentricity B of the release agent domain becomes smaller.

For example, the skewness in the distribution of the eccentricity B of the release agent domain is adjusted depending on a period of time when the dispersions are respectively transported from the second storage tank 322 and the third storage tank 323, and a liquid transport speed at which the dispersion is transported to the first storage tank 321 from the second storage tank 322. More specifically, for example, if a liquid transport starting time of the release agent particle dispersion from the third storage tank 323 and a liquid transport starting time of the dispersion from the second storage tank 322 are early, and the liquid transport speed of the dispersion from the second storage tank 322 is lowered, a state where the release agent particles are disposed from a further inner side of the formed aggregated particle to a further outer side thereof is realized. Thus, the

skewness in the distribution of the eccentricity B of the release agent domain becomes greater.

For example, the kurtosis in the distribution of the eccentricity B of the release agent domain is adjusted by changing the liquid transport speed of the release agent particle dispersion from the third storage tank 323 in the process of liquid transport. More specifically, for example, if only the liquid transport speed of the release agent particle dispersion from the third storage tank 323 becomes faster in the process of liquid transport, the concentration of the release agent particles in the dispersion of the second storage tank 322 becomes higher from that time. For this reason, there arises a state where many of the release agent particles are disposed in a certain area (certain deep portion) in a radial direction of the aggregated particle in the formed aggregated particle. Thus, the kurtosis in the distribution of the eccentricity B of the release agent domain becomes greater.

The above-described power feeding addition method is not limited to the above method. For example, various methods may be employed. Examples of the various methods include a method in which, a storage tank storing the second resin particle dispersion and a storage tank storing a dispersion mixture in which the second resin particles and the release agent particles are dispersed are separately provided and the respective dispersions are transported to the first storage tank 321 from the respective storage tanks while changing the liquid transport speed, a method in which a storage tank storing the release agent particle dispersion and a storage tank storing a dispersion mixture in which the second resin particles and the release agent particles are dispersed are separately provided, and the respective dispersions are transported to the first storage tank 321 from the respective storage tanks while changing the liquid transport speed, and the like.

As described above, the second aggregated particles in which the second resin particles and the release agent particles are attached to the surfaces of the first aggregated particles and aggregated are obtained.

#### Coalescence Process

Next, the second aggregated particle dispersion in which the second aggregated particles are dispersed is heated at, for example, a temperature that is equal to or higher than the glass transition temperature of the first and second resin particles (for example, a temperature that is higher than the glass transition temperature of the first and second resin particles by 10° C. to 30° C.) to coalesce the second aggregated particles and form toner particles.

The toner particles are obtained through the above-described processes.

Furthermore, the toner particles may be prepared as follows. That is, after the aggregated particle dispersion in which the second aggregated particles are dispersed is obtained, toner particles may be prepared through the processes of:

further mixing the second aggregated particle dispersion with a third resin particle dispersion in which third resin particles corresponding to the binder resin are dispersed to perform aggregation so that the third resin particles further adhere to the surfaces of the second aggregated particles, thereby forming third aggregated particles; and coalescing the third aggregated particles by heating the third aggregated particle dispersion in which the third aggregated particles are dispersed, and thereby forming toner particles having a core/shell structure.

With respect to the toner particles prepared according to the processes, the maximum frequent value in the distribution of the eccentricity B of the release agent domain is less than 1.00.

After the coalescence process is ended, toner particles formed in a solution are subjected to a well-known washing process, a well-known solid-liquid separation process, a well-known drying process, and thereby dried toner particles are obtained.

Regarding the washing process, replacing washing using ion exchanged water may preferably be sufficiently performed for charging property. The solid-liquid separation process is not particularly limited, but suction filtration, pressure filtration, or the like may preferably be performed for productivity. The drying process is not particularly limited, but freeze drying, flash jet drying, fluidized drying, vibrating fluidized drying, and the like may preferably be performed for productivity.

The toner in this exemplary embodiment is prepared, for example, by adding an external additive to the obtained toner particles in a dried state, and performing mixing. The mixing may be performed, for example, by using a V blender, a HENSCHEL mixer, a Lödige mixer, or the like. Furthermore, if necessary, coarse toner particles may be removed using a vibration sieving machine, a wind classifier, or the like.

#### Electrostatic Charge Image Developer

An electrostatic charge image developer according to this exemplary embodiment contains at least the toner in this exemplary embodiment.

The electrostatic charge image developer according to this exemplary embodiment may be a single-component developer which contains only the toner in this exemplary embodiment, or be a two-component developer obtained by mixing the toner with a carrier.

The carrier is not particularly limited, and known carriers are exemplified. Examples of the carrier include a coated carrier in which surface of core formed of a magnetic powder is coated with a coating resin; a magnetic powder dispersion-type carrier in which a magnetic powder is dispersed and blended in a matrix resin; and a resin impregnation-type carrier in which a porous magnetic powder is impregnated with a resin.

The magnetic powder dispersion-type carrier and the resin impregnation-type carrier may be carriers in which constituent particles of the carrier are cores and coated with a coating resin.

Examples of the magnetic powder include magnetic metals such as iron, nickel, and cobalt, and magnetic oxides such as ferrite and magnetite.

Examples of the coating resin and the matrix resin include polyethylene, polypropylene, polystyrene, polyvinyl acetate, polyvinyl alcohol, polyvinyl butyral, polyvinyl chloride, polyvinyl ether, polyvinyl ketone, a vinyl chloride-vinyl acetate copolymer, a styrene-acrylic acid copolymer, a straight silicone resin configured to include an organosiloxane bond or a modified product thereof, a fluororesin, polyester, polycarbonate, a phenol resin, and an epoxy resin.

The coating resin and the matrix resin may contain other additives such as conductive particles.

Examples of the conductive particles include particles of metal such as gold, silver, and copper, and particles of carbon black, titanium oxide, zinc oxide, tin oxide, barium sulfate, aluminum borate, potassium titanate, and the like.

Here, a coating method using a coating layer forming solution in which a coating resin, and if necessary, various additives are dissolved in an appropriate solvent is used to

coat the surface of a core with the coating resin. The solvent is not particularly limited, and may be selected in consideration of the coating resin to be used, coating suitability, and the like.

Specific examples of the resin coating method include a dipping method of dipping cores in a coating layer forming solution, a spraying method of spraying a coating layer forming solution to surfaces of cores, a fluid bed method of spraying a coating layer forming solution in a state in which cores are allowed to float by flowing air, and a kneader-coater method in which cores of a carrier and a coating layer forming solution are mixed with each other in a kneader-coater and the solvent is removed.

The mixing ratio (weight ratio) between the toner and the carrier in the two-component developer is preferably from 1:100 to 30:100, and more preferably from 3:100 to 20:100 (toner:carrier).

#### Image Forming Apparatus/Image Forming Method

Next, the configuration of the image forming apparatus (configuration of the image forming method) according to this exemplary embodiment will be described.

As the image forming apparatus according to this exemplary embodiment, a well-known image forming apparatus is applied. Examples of the well-known image forming apparatus include a direct transfer type apparatus that directly transfers a toner image formed on a surface of an image holding member to a recording medium; an intermediate transfer type apparatus that primarily transfers a toner image formed on a surface of an image holding member to a surface of an intermediate transfer member, and secondarily transfers the toner image which has been transferred onto the surface of the intermediate transfer member to a surface of a recording medium; an apparatus including a cleaning unit that cleans a surface of an image holding member after transferring of a toner image and before charging; and an apparatus including an erasing unit that performs erasing by irradiating a surface of an image holding member with eraser light after transferring of a toner image and before charging.

In a case of the intermediate transfer type apparatus, for example, a configuration is applied in which a transfer unit includes an intermediate transfer member onto the surface of which the toner image is transferred, a primary transfer unit that primarily transfers the toner image formed on the surface of the image holding member onto a surface of the intermediate transfer member, and a secondary transfer unit that secondarily transfers the toner image which has been transferred onto the surface of the intermediate transfer member onto the surface of a recording medium.

In the image forming apparatus according to this exemplary embodiment, for example, a part including the developing unit may be a cartridge structure (process cartridge) which is detachable from the image forming apparatus. As the process cartridge, for example, a process cartridge which includes a developing unit storing an electrostatic charge image developer used in this exemplary embodiment is appropriately used.

In the image forming apparatus according to this exemplary embodiment, the fixing method (multi-stage fixing method) is employed in which the heating and pressing member contacts with a toner image on a recording medium twice or more and the heating and pressing operation is performed twice or more. Particularly, in view of improving gloss of an image, the multi-stage fixing method in which the first heating and pressing operation serves a fixing function, and the second heating and pressing operation serves a gloss improvement function is preferable. For

21

example, since as the thickness of a recording medium becomes thicker, improvement of gloss of an image becomes more difficult, an effect of improvement of gloss obtained by using the above-described multi-stage fixing method is shown more.

An example of the image forming apparatus according to this exemplary embodiment will be described below. However, it is not limited thereto. Main components illustrated in the drawings will be described and descriptions of other components will be omitted.

FIG. 1 is a schematic configuration diagram illustrating the image forming apparatus according to this exemplary embodiment.

The image forming apparatus illustrated in FIG. 1 includes first to fourth electrophotographic image forming units **10Y**, **10M**, **10C**, and **10K** (image forming units) that respectively print yellow (Y), magenta (M), cyan (C), and black (K) images based on color-separated image data. These image forming units (which may be simply referred to as "units" below) **10Y**, **10M**, **10C**, and **10K** are arranged side by side at predetermined intervals in a horizontal direction. These units **10Y**, **10M**, **10C**, and **10K** may be process cartridges that are detachable from the image forming apparatus.

An intermediate transfer belt **20** as an intermediate transfer member is installed above the units **10Y**, **10M**, **10C**, and **10K** in the drawing so as to extend through the units. The intermediate transfer belt **20** is wound on a driving roller **22** and a support roller **24** contacting the inner surface of the intermediate transfer belt **20**, which are separated from each other on the left and right sides in the drawing, and the intermediate transfer belt **20** travels in a direction toward the fourth unit **10K** from the first unit **10Y**. A force is applied to the support roller **24** in a direction in which it departs from the driving roller **22** by a spring or the like (not illustrated), and a tension is applied to the intermediate transfer belt **20** wound on both of the rollers. In addition, an intermediate transfer member cleaning device **30** is provided on a surface of the intermediate transfer belt **20** on the photoreceptor side so as to face the driving roller **22**.

The developers including toners of four colors are respectively stored in developing devices (one example of developing units) **4Y**, **4M**, **4C**, and **4K** of the units **10Y**, **10M**, **10C**, and **10K**. Further, a yellow toner, a magenta toner, a cyan toner, and a black toner contained in toner cartridges **8Y**, **8M**, **8C**, and **8K** are respectively supplied to the developing devices **4Y**, **4M**, **4C**, and **4K**.

The first to fourth units **10Y**, **10M**, **10C**, and **10K** have the same configuration. Thus, only the first unit **10Y** that is disposed on the upstream side in a traveling direction of the intermediate transfer belt and forms a yellow image will be representatively described here. The same parts as in the first unit **10Y** will be denoted by the reference numerals with magenta (M), cyan (C), and black (K) added instead of yellow (Y), and descriptions of the second to fourth units **10M**, **10C**, and **10K** will be omitted.

The first unit **10Y** includes a photoreceptor **1Y** as the image holding member. Around the photoreceptor **1Y**, a charging roller (an example of the charging unit) **2Y**, an exposure device (an example of the electrostatic charge image forming unit) **3**, a developing device (an example of the developing unit) **4Y**, a primary transfer roller (an example of the primary transfer unit) **5Y**, and a photoreceptor cleaning device (an example of the cleaning unit) **6Y** are arranged in sequence. The charging roller **2Y** charges a surface of the photoreceptor **1Y** to a predetermined potential. The exposure device **3** exposes the charged surface with

22

laser beams **3Y** based on a color-separated image signal to form an electrostatic charge image. The developing device **4Y** supplies a charged toner to the electrostatic charge image to develop the electrostatic charge image. The primary transfer roller **5Y** transfers the developed toner image onto the intermediate transfer belt **20**. The photoreceptor cleaning device **6Y** removes the toner remaining on the surface of the photoreceptor **1Y** after primary transfer.

The primary transfer roller **5Y** is provided inside the intermediate transfer belt **20** to be provided at a position facing the photoreceptor **1Y**. Bias supplies (not illustrated) that apply a primary transfer bias are respectively connected to the primary transfer devices **5Y**, **5M**, **5C**, and **5K**. Each of the bias supplies changes a transfer bias that is applied to each of the primary transfer rollers, under a control by a control unit (not illustrated).

An example of an operation of forming a yellow image by the first unit **10Y** will be described below.

First, before the operation, the surface of the photoreceptor **1Y** is charged by the charging roller **2Y** so as to have a potential from -600 V to -800 V.

The photoreceptor **1Y** is formed by laminating a photosensitive layer on a conductive (for example, volume resistivity at 20° C.:  $1 \times 10^{-6} \Omega \text{cm}$  or less) substrate. The photoreceptor **1Y** has properties in which resistance is normally high (resistance of a general resin), but the specific resistance of a portion irradiated with the laser beams changes when the laser beams **3Y** are applied. Thus, the laser beams **3Y** is output to the charged surface of the photoreceptor **1Y** through the exposure device **3** in accordance with image data for yellow transmitted from the control unit (not illustrated). The photosensitive layer on the surface of the photoreceptor **1Y** is irradiated with the laser beams **3Y**, and thereby an electrostatic charge image of a yellow image pattern is formed on the surface of the photoreceptor **1Y**.

The electrostatic charge image is an image which is formed on the surface of the photoreceptor **1Y** by charging, and is a so-called negative latent image, which is formed by applying the laser beams **3Y** to the photosensitive layer so that the specific resistance of the irradiated part is decreased to cause charges on the surface of the photoreceptor **1Y** to flow while charges stay on a part to which the laser beams **3Y** are not applied.

The electrostatic charge image formed on the photoreceptor **1Y** is rotated up to a predetermined developing position with the travelling of the photoreceptor **1Y**. The electrostatic charge image on the photoreceptor **1Y** is visualized (developed) as a toner image at this developing position by the developing device **4Y**.

The developing device **4Y** stores, for example, an electrostatic charge image developer including at least a yellow toner and a carrier. The yellow toner is frictionally charged by performing stirring in the developing device **4Y** and has charges with the same polarity (negative polarity) as the charges which are generated on the photoreceptor **1Y**. Thus, the yellow toner is held on a developer roller (an example of a developer holding member). The surface of the photoreceptor **1Y** is allowed to pass through the developing device **4Y**, and thus the yellow toner electrostatically adheres to an electrostatic latent image portion erased on the surface of the photoreceptor **1Y**, and thereby the latent image is developed by using the yellow toner. The photoreceptor **1Y** having the yellow toner image formed thereon continuously travels at a predetermined speed and the toner image developed on the photoreceptor **1Y** is transported to a predetermined primary transfer position.

When the yellow toner image on the photoreceptor 1Y is transported to the primary transfer position, a primary transfer bias is applied to the primary transfer roller 5Y and an electrostatic force toward the primary transfer roller 5Y from the photoreceptor 1Y acts on the toner image, and thereby the toner image on the photoreceptor 1Y is transferred onto the intermediate transfer belt 20. The transfer bias applied at this time has the opposite polarity (+) to the polarity (-) of the toner, and, for example, is controlled so as to be +10  $\mu$ A in the first unit 10Y by the controller (not illustrated).

The residual substances remaining on the photoreceptor 1Y are removed by the photoreceptor cleaning device 6Y, and a toner of the residual substances is collected.

The primary transfer biases which are applied to the primary transfer rollers 5M, 5C, and 5K of the second unit 10M and the subsequent units are also controlled similarly to a case of the first unit.

In this manner, the intermediate transfer belt 20 onto which the yellow toner image is transferred in the first unit 10Y is sequentially transported through the second to fourth units 10M, 10C, and 10K, and the toner images of respective colors are multiply-transferred in a superimposed manner.

The four color toner images which have been multiply-transferred onto the intermediate transfer belt 20 through the first to fourth units reach a secondary transfer part that is made of the intermediate transfer belt 20, the support roller 24 contacting the inner surface of the intermediate transfer belt, and a secondary transfer roller (an example of the secondary transfer unit) 26 disposed on the image holding surface side of the intermediate transfer belt 20.

A recording sheet (an example of the recording medium) P is fed to a gap between the secondary transfer roller 26 and the intermediate transfer belt 20, which contact with each other, through a supply mechanism at a predetermined timing, and a secondary transfer bias is applied to the support roller 24. The transfer bias applied at this time has the same polarity (-) as the polarity (-) of the toner. An electrostatic force toward the recording sheet P from the intermediate transfer belt 20 acts on the toner image, and thereby the toner image of four colors on the intermediate transfer belt 20 is transferred onto the recording sheet P. In this case, the secondary transfer bias is determined depending on the resistance detected by a resistance detector (not illustrated) that detects the resistance at the secondary transfer position, and is voltage-controlled.

Then, the recording sheet P is supplied to the fixing device (an example of the fixing unit) 28 and the toner image is fixed onto the recording sheet P, and thereby a fixation image is formed. In this exemplary embodiment, the fixing method (multi-stage fixing method) is employed in which the heating and pressing member contacts with the toner image on the recording medium twice or more, thereby performing the heating and pressing operation twice or more.

FIGS. 1 and 2 illustrate an example of the multi-stage fixing type fixing device in which fixing is performed by performing the heating and pressing operation twice. The reference numerals 91a and 91b are a pair of fixing rolls in the first operation (an example of the heating and pressing member in the first operation). A recording sheet P on which an unfixed toner image is had is fed in a direction of an arrow E, and passes through between the pair of fixing rolls 91a and 91b. The toner image is heated and first fixing is performed.

Then, the recording sheet P subjected to the first fixing passes through a pair of second fixing rolls 92a and 92b (an example of the second heating and pressing member), and second fixing is performed by further heating and pressing

the fixed toner image. Particularly, it is preferable that the second fixing causes the gloss of an image to be improved.

Here, a configuration of the pair of fixing rolls will be described.

The fixing rolls 91b and 92b which directly contact with a toner image are formed to have a cylindrical shape, for example. The toner image is fixed to the recording sheet P by causing the outermost layers of the fixing rolls 91b and 92b to contact with a toner image surface of the recording sheet P so as to heat and press the toner image surface. The fixing rolls 91b and 92b may have, for example, a multi-layer structure in which a core roll and an elastic layer are provided outwardly from the inner side of the fixing roll in a radial direction thereof. An outermost layer may be further provided on the outside of the elastic layer.

The core roll is a cylindrical member and supports the elastic layer and the outermost layer which are disposed on an outer circumferential surface. For example, the core roll has a configuration in which hubs (portions to which bearings are attached) made of SUS (stainless steel) are provided at both end portions of an aluminum alloy pipe member in an axial direction. The material of the core roll is not limited thereto, and the core roll may be formed of other materials. Examples of the material of the core roll include metal such as aluminum (material A-5052, and the like), iron, SUS, and copper, alloy, ceramics, fiber reinforced metal (FRM), and the like. In addition, the core roll may be formed of a resin. The shape of the core roll is not limited to the cylindrical (hollow) shape, and may be a columnar (solid) shape.

Examples of a material of the elastic layer include urethane rubber, ethylene propylene rubber (EPM), silicone rubber, fluororubber (FKM), and the like. Particularly, silicone rubber having excellent thermal resistance and excellent processability is included. Examples of the silicone rubber include RTV silicone rubber, HTV silicone rubber, and the like. Specific examples include polydimethyl silicone rubber (MQ), methylvinyl silicone rubber (VMQ), methylphenyl silicone rubber (PMQ), fluoro silicone rubber (FVMQ), and the like.

An adhesive layer may be provided between the core roll and the elastic layer. An outermost layer may be further provided on the outside of the elastic layer.

In the fixing rolls 91b and 92b, a halogen heater may be provided on an inner side as an inner heat applying unit. The halogen heater generates heat by electrification from a power source and heats the fixing rolls 91b and 92b from the inside.

A cleaning web may contact with the outer circumferential surface of the fixing rolls 91b and 92b so as to remove the release agent adhering to the outer circumferential surface of the fixing rolls 91b and 92b.

The fixing rolls 91a and 92a which do not directly contact with the toner image are formed to have a cylindrical shape. The toner image is fixed to the recording sheet P by causing the outermost layers of the fixing rolls 91a and 92a to contact with a surface of the recording sheet P on an opposite side of the toner image surface so as to perform pressing (or heating and pressing). The fixing rolls 91a and 92a may have, for example, a multi-layer structure in which a core roll and an elastic layer are provided outwardly from the inner side of the fixing roll in a radial direction thereof. An outermost layer may be provided on the outside of the elastic layer. The fixing rolls 91a and 92a may be pushed toward the fixing rolls 91b and 92b by using a pushing unit such as a spring. As the core roll and the elastic layer, a core roll and an elastic layer which are the same as those described for fixing rolls 91b and 92b are preferably exemplified. An inner

heat applying unit such as a halogen heater may be provided on an inner side of the fixing rolls 91a and 92a.

The descriptions are made with reference to the drawing for an aspect using the two pairs of fixing rolls as an example of the multi-stage fixing type fixing device. However, the multi-stage fixing type fixing device in this exemplary embodiment is not limited thereto. For example, as the heating and pressing member, a heating and pressing member in which a roll-shaped rotation member and a belt-shaped rotation member constituting a pair contact with each other so as to form a nip, and a recording sheet to which a toner image is transferred is inserted into the nip may be used. In addition, as the heating and pressing member, a heating and pressing member in which two belt-shaped rotation members constituting a pair contact with each other so as to form a nip may be used.

The number of heating and pressing members is not limited to 2, and three or more heating and pressing members may be used.

In addition to an aspect in which two or more heating and pressing members are provided and a recording sheet passes through each of the plural heating and pressing members once, an aspect in which one heating and pressing member is provided and a recording sheet passes through the heating and pressing member twice or more repeatedly may be employed.

Examples of the recording sheet P onto which the toner image is transferred include plain paper used in an electro-photographic copying machine, a printer, and the like. The recording medium includes an OHP sheet and the like in addition to the recording sheet P.

In order to improve smoothness of an image surface after fixing, the surface of the recording sheet P is preferably also smooth. For example, coated paper obtained by coating a surface of plain paper with a resin and the like, or art paper for printing is appropriately used.

The recording sheet P on which fixing of the color image is completed is discharged toward a discharge unit, and a series of the color image forming operations is ended.

## EXAMPLES

This exemplary embodiment will be described more specifically in detail by using examples and comparative examples. However, this exemplary embodiment is not limited these examples. A "part" means a "part by weight" unless otherwise indicated.

### Preparation of Resin Particle Dispersion

#### Preparation of Resin Particle Dispersion (1)

30 parts by mol of terephthalic acid, 70 parts by mol of fumaric acid, 5 parts by mol of an ethylene oxide adduct of bisphenol A, and 95 parts by mol of a propylene oxide adduct of bisphenol A are put into a 5-liter flask provided with a stirrer, a nitrogen inlet tube, a thermometer, and a rectifying column. The temperature of the flask is increased up to 210° C. over one hour, and 1 part of titanium tetrabutoxide relative to 100 parts of the materials is put into the flask. The temperature is increased up to 230° C. over 0.5 hours while generated water is distilled away. After a dehydration condensation reaction is continued at that temperature for one hour, the reactant is cooled. In this manner, Polyester resin (1) having a weight-average molecular weight of 18,500, an acid value of 14 mgKOH/g, and a glass transition temperature of 59° C. is synthesized.

40 parts of ethyl acetate and 25 parts of 2-butanol are put into a container provided with a temperature adjusting unit and a nitrogen substituting unit to obtain a mixed solvent.

Then, 100 parts of Polyester resin (1) are slowly put into the mixed solvent to thereby be dissolved. 10% by weight of an ammonia aqueous solution (having an amount corresponding to three times an acid value of the resin in a molar ratio) is put into the obtained mixture, followed by stirring for 30 minutes.

Then, substitution with dry nitrogen is performed in the container, and the temperature is held at 40° C. 400 parts of ion-exchanged water are dropped into the liquid mixture at a speed of 2 parts/minute while stirring to prepare an emulsion. After dropping is ended, the temperature of the emulsion is returned to the room temperature (20° C. to 25° C.), and bubbling is performed for 48 hours by using dry nitrogen while stirring such that ethyl acetate and 2-butanol are reduced to be equal to or less than 1,000 ppm. Thus, a resin particle dispersion in which resin particles having a volume average particle diameter of 200 nm are dispersed is obtained. Ion-exchanged water is added to the resin particle dispersion so as to adjust a solid content to be 20% by weight, and the obtained dispersion is used as Resin particle dispersion (1).

### Preparation of Colorant Particle Dispersion

#### Preparation of Colorant Particle Dispersion (1)

70 parts of a cyan pigment: C.I. Pigment Blue 15:3 (copper phthalocyanine, product manufactured by DIC Corporation, product name: FASTOGEN BLUE LA5380), 5 parts of anionic surfactant (NEOGEN RK, product manufactured by DKS Co., Ltd.,), and 200 parts of ion-exchanged water are mixed with each other, and are dispersed by using a homogenizer (ULTRA-TURRAX T50, product manufactured by IKA Corporation) for 10 minutes. Ion-exchanged water is added so as to cause a solid content in the dispersion to be 20% by weight, and thereby Colorant particle dispersion (1) in which colorant particles having a volume average particle diameter of 190 nm are dispersed is obtained.

### Preparation of Release Agent Particle Dispersion

#### Preparation of Release Agent Particle Dispersion (1)

100 parts of a paraffin wax (HNP-9, product manufactured by NIPPON SEIRO Co., Ltd.), 1 part of an anionic surfactant (NEOGEN RK, product manufactured by DKS Co., Ltd.), 350 parts of ion-exchanged water are mixed with each other, heated up to 100°, and dispersed by using a homogenizer (ULTRA-TURRAX T50, product manufactured by IKA Corporation). Then, dispersing is performed by using a Manton-Gaulin high-pressure homogenizer (product manufactured by Gaulin Corporation), to thereby obtain Release agent particle dispersion (1) (solid content of 20% by weight) in which release agent particles having a volume average particle diameter of 200 nm are dispersed.

### Preparation of Developer (1)

#### Preparation of Toner Particle (1)

An apparatus (see FIG. 3) having the following configuration is prepared: a round stainless steel flask and a container A are connected to each other by using a tube pump A; driving of the tube pump A causes a liquid stored in the container A is transported to the flask; the container A and a container B are connected to each other by using a tube pump B; driving of the tube pump B causes a liquid stored in the container B to be transported to the container A. The following operations are performed by using this apparatus.

500 parts of Resin particle dispersion (1), 40 parts of Colorant particle dispersion (1), and 2 parts of an anionic surfactant (TAYCAPOWER) are put into a round stainless steel flask, and 0.1 N nitric acid is added to the liquid so as to adjust the pH of the liquid to 3.5. Then, 30 parts of a nitric acid aqueous solution in which a concentration of polyaluminum chloride is 10% by weight are added thereto. Sub-

sequently, the obtained mixture is dispersed at 30° C. by using a homogenizer (ULTRA-TURRAX T50, product manufactured by IKA Corporation), and then, the temperature of the obtained dispersion is increased at a pace of 1° C./30 minutes in an oil bath for heating to thereby increase a particle diameter of aggregated particles.

150 parts of Resin particle dispersion (1) are put into the container A which is a bottle made of a polyester, and 25 parts of Release agent particle dispersion (1) are put into the container B which is a bottle made of a polyester. Then, a liquid transport speed of the tube pump A is set to 0.70 parts/1 minute, and a liquid transport speed of the tube pump B is set to 0.14 parts/1 minute. The tube pumps A and B are driven from a point of time when the temperature of the inside of the round stainless steel flask in the process of forming of the aggregated particle reaches 37.0° C., and thus transporting of the respective dispersions is started. Accordingly, a dispersion mixture in which resin particles and release agent particles are dispersed is transported from the container A to the round stainless steel flask which is in the process of forming of the aggregated particle, with a gradual increase of the concentration of the release agent particles.

The content of the flask is held for 30 minutes from a point of time when the temperature of the inside of the flask is 48° C. after transporting of the dispersions to the flask is ended, and thereby second aggregated particles are formed.

Then, 50 parts of Resin particle dispersion (1) are added slowly and the obtained mixture is held for 1 hour. 0.1 N sodium hydroxide aqueous solution is added thereto to thereby adjust the pH of the mixture to 8.5. Then, heating is performed up to 85° C. with continuous stirring, and the resultant is held for 5 hours. Then, the resultant is cooled to 20° C. at a speed of 20° C./minute, is filtered, is sufficiently washed by using ion-exchanged water, and then is dried. Thus, Toner particles (1) having a volume average particle diameter of 6.0  $\mu\text{m}$  are obtained.

#### Preparation of Toner (1)

100 parts of Toner particles (1), 0.7 parts of dimethyl silicone oil-treated silica particles (RY200, product manufactured by NIPPON AEROSIL CO., LTD.) are mixed with each other by using a HENSCHEL mixer (peripheral speed of 30 m/s, 3 minutes), and thereby Toner (1) is obtained.

#### Preparation of Developer (1)

Among 100 parts of ferrite particles (average particle diameter of 50  $\mu\text{m}$ ), 14 parts of toluene, 3 parts of a styrene/methyl methacrylate copolymer (copolymerization ratio: 15/85), and 0.2 parts of carbon black, the components except for the ferrite particles are dispersed in a sand mill to thereby prepare a dispersion. This dispersion and the ferrite particles are put into a vacuum degassing kneader. Decompression and drying is performed with stirring to thereby obtain a carrier.

8 parts of Toner (1) are mixed with 100 parts of the carrier, and thereby Developer (1) is obtained.

#### Comparative Example 1

##### Preparation of Comparative Developer (1)/Toner of which the Release Agent Unevenly Exists Only in the Inside

Toner Particles (C1) are obtained in the same manner as the preparation of Toner Particles (1) in Example 1 except that the liquid transport speed of the tube pump A is set to 0.84 parts/1 minute, the liquid transport speed of the tube pump B is set to 0.17 parts/1 minute, and the tube pumps A and B are driven from a point of time when the temperature of the inside of the flask reaches 33.0° C. Toner Particles (C1) which are obtained has a volume average particle

diameter of 6.0  $\mu\text{m}$ . In the same manner as in Example 1, Toner (C1) is prepared by using Toner particles (C1), and Comparative Developer (1) is obtained by using Toner (C1).

#### Comparative Example 2

##### Preparation of Comparative Developer (2)/Toner of which the Release Agent Unevenly Exists Only at the Surface Portion

Toner Particles (C2) are obtained in the same manner as the preparation of Toner Particles (1) in Example 1 except that the liquid transport speed of the tube pump A is set to 0.89 parts/1 minute, the liquid transport speed of the tube pump B is set to 0.19 parts/1 minute, and the tube pumps A and B are driven from a point of time when the temperature of the inside of the flask reaches 42.0° C. Toner Particles (C2) which are obtained has a volume average particle diameter of 5.5  $\mu\text{m}$ . In the same manner as in Example 1, Toner (C2) is prepared by using Toner particles (C2), and Comparative Developer (2) is obtained by using Toner (C2).

#### Various Measurements

Regarding the toner of the developer obtained in each of the examples, the maximum frequent value, the skewness, and the kurtosis in the distribution of the eccentricity B of the release agent domain are measured by using the above-described method. The results are shown in Table 1.

#### Evaluation

Evaluation is performed as follows by using the developer obtained in each of the examples. The results are shown in Table 1.

As an image forming apparatus for forming an evaluation image, a modified machine (product manufactured by Fuji Xerox Co., Ltd., product name: D136P) (image forming apparatus including a multi-stage fixing type fixing machine illustrated in FIG. 2) is prepared. A developer is put into a developing machine and a replenishing toner (the same toner as a toner contained in the developer) is put into a toner cartridge. Then, an image which includes a band-shaped solid image having a width of 100 mm, a length of 400 mm is printed on a thick seat of paper (product manufactured by Fuji Xerox Co., Ltd., product name: NCOLOR209GSM) to thereby provide 100,000 pieces of paper having a printed image.

#### Evaluation of Offset (Toner Adhesion)

A degree of occurrence of offset to the first pair of fixing rolls (heating and pressing member) and occurrence of offset to the second pair of fixing rolls (heating and pressing member) is evaluated based on the following evaluation standards by observing a scattering state at a position corresponding to a position of the fixing roll at which the band image is formed.

A: no difference in a scattering state in comparison to a portion of no band image

B: presence of a difference in a scattering state in comparison to a portion of no band image

#### Evaluation of Gloss of Image

The gloss of the last printed image is measured by an evaluating apparatus (Micro-TRI gloss meter (60° gloss), manufactured by BYK Gartner Inc.).

TABLE 1

| Developer   | Distribution of eccentricity B of release agent domain |          |          | Evaluation |        |       |
|-------------|--------------------------------------------------------|----------|----------|------------|--------|-------|
|             | Maximum                                                |          |          | Offset     |        |       |
|             | frequent value                                         | Skewness | Kurtosis | First      | Second | Gloss |
| Example 1   | Developer (1)                                          | 0.88     | -0.80    | 0.60       | A      | 2.5   |
| Comparative | Comparison                                             | 0.74     | -0.52    | 0.63       | A      | 1.5   |
| Example 1   | developer (1)                                          |          |          |            |        |       |
| Comparative | Comparison                                             | 0.99     | -0.47    | 0.59       | A      | 2.0   |
| Example 2   | developer (2)                                          |          |          |            |        |       |

It is confirmed based on the result that adhering (offset) of the toner to the heating and pressing member is prevented in the multi-stage fixing method, in this example in comparison to the comparative examples. In addition, it is confirmed that good gloss is obtained for an image.

The foregoing description of the exemplary embodiments of the present invention has been provided for the purposes of illustration and description. It is not intended to be exhaustive or to limit the invention to the precise forms disclosed. Obviously, many modifications and variations will be apparent to practitioners skilled in the art. The embodiments were chosen and described in order to best explain the principles of the invention and its practical applications, thereby enabling others skilled in the art to understand the invention for various embodiments and with the various modifications as are suited to the particular use contemplated. It is intended that the scope of the invention be defined by the following claims and their equivalents.

What is claimed is:

1. An image forming apparatus comprising:  
an image holding member;  
a charging unit that charges a surface of the image holding member;  
an electrostatic charge image forming unit that forms an electrostatic charge image on a charged surface of the image holding member;  
a developing unit that stores a developer containing a toner and develops the electrostatic charge image formed on a surface of the image holding member by using the developer so as to form a toner image;  
a transfer unit that transfers the toner image formed on the surface of the image holding member onto a surface of a recording medium; and  
a fixing unit that performs an operation of heating and pressing to the toner image on the recording medium twice or more by using one or more of a heating and pressing member which contacts with the toner image, wherein the toner contains a binder resin, a colorant, and a release agent, and has a sea and island structure of a sea portion containing the binder resin and an island portion containing the release agent,  
a maximum frequent value in distribution of an eccentricity B of the island portion containing the release agent is in a range of from 0.75 to 0.95, and  
a skewness in the distribution of the eccentricity B is in a range of from -1.10 to -0.50,  
the eccentricity B being represented by the following expression (1):

$$\text{Eccentricity } B=2d/D \quad (1)$$

wherein D indicates an equivalent circle diameter ( $\mu\text{m}$ ) of the toner in an observation of a cross-section of the toner, and d indicates a distance ( $\mu\text{m}$ ) from the centroid

of the toner to the centroid of the island portion containing the release agent in the observation of a cross-section of the toner, and  
wherein the release agent is a paraffin wax, and the binder resin is a polyester resin.

2. The image forming apparatus according to claim 1, wherein a kurtosis of the distribution of the eccentricity B in the toner is in a range of from -0.20 to +1.50.

3. The image forming apparatus according to claim 1, wherein the maximum frequent value in the distribution of the eccentricity B in the toner is in a range of from 0.80 to 0.90.

4. The image forming apparatus according to claim 1, wherein a kurtosis of the distribution of the eccentricity B in the toner is in a range of from -0.10 to +1.40.

5. The image forming apparatus according to claim 1, wherein the fixing unit performs an operation of heating and pressing for fixing and an operation of heating and pressing for gloss control of an image.

6. An image forming method comprising:  
charging a surface of an image holding member;  
forming an electrostatic latent image on a charged surface of the image holding member;  
developing the electrostatic latent image formed on the surface of the image holding member by using a developer containing a toner so as to form a toner image;  
transferring the toner image to a surface of a recording medium; and  
fixing the toner image by performing an operation of heating and pressing the toner image on the recording medium twice or more, with one or more of a heating and pressing member which contacts with the toner image,

wherein the toner contains a binder resin, a colorant, and a release agent, and has a sea and island structure of a sea portion containing the binder resin and an island portion containing the release agent,

a maximum frequent value in distribution of an eccentricity B of the island portion containing the release agent is in a range of from 0.75 to 0.95, and  
a skewness in the distribution of the eccentricity B is in a range of from -1.10 to -0.50,  
the eccentricity B being represented by the following expression (1):

$$\text{Eccentricity } B=2d/D \quad (1)$$

wherein D indicates an equivalent circle diameter ( $\mu\text{m}$ ) of the toner in an observation of a cross-section of the toner, and d indicates a distance ( $\mu\text{m}$ ) from a centroid of the toner to a centroid of the island portion containing the release agent in the observation of a cross-section of the toner.

**31**

7. The image forming method according to claim 6, wherein a kurtosis of the distribution of the eccentricity B in the toner is in a range of from -0.20 to +1.50.

8. The image forming method according to claim 6, wherein the maximum frequent value in the distribution of the eccentricity B in the toner is in a range of from 0.80 to 0.90. 5

9. The image forming method according to claim 6, wherein a kurtosis of the distribution of the eccentricity B in the toner is in a range of from -0.10 to +1.40. 10

10. The image forming method according to claim 6, wherein the fixing is performed by an operation of heating and pressing for fixing and an operation of heating and pressing for gloss control of an image. 15

11. An image forming apparatus comprising:

a multi-stage fixing unit comprising one or more of a heating and pressing member, the multi-stage fixing unit performing a multi-stage fixing process of heating

**32**

and pressing a toner image formed on a recording medium using the one or more of the heating and pressing member,

wherein the toner contains a binder resin, a colorant, and a release agent, and has a sea and island structure of a sea portion containing the binder resin and an island portion containing the release agent,

wherein an eccentricity B of the island portion containing the release agent is given by  $B=2d/D$ , wherein D denotes an equivalent circle diameter ( $\mu\text{m}$ ) of the toner in a cross-section of the toner, and d denotes a distance ( $\mu\text{m}$ ) from the centroid of the toner to the centroid of the island portion containing the release agent in the cross-section of the toner,

wherein a distribution of the eccentricity B forms a bell-shaped curve having a maximum value in a range of from 0.75 to 0.95, and a skewness in a range of from -1.10 to -0.50.

\* \* \* \* \*